

[72] Inventors Keisuke Shiba;  
Masanao Hinata; Hiroshi Misu; Masao  
Sawahara, all of Kanagawa, Japan

[21] Appl. No. 707,478

[22] Filed Feb. 23, 1968

[45] Patented Nov. 2, 1971

[73] Assignee Fuji Photo Film Co., Ltd.  
Kanagawa, Japan

[32] Priority Feb. 23, 1967

[33] Japan

[31] 42/11669

[54] PHOTOGRAPHIC SILVER HALIDE EMULSION  
8 Claims, No Drawings

[52] U.S. Cl. 96/126,  
96/109

[51] Int. Cl. G03c 1/28

[50] Field of Search 96/104, 109

[56] References Cited

UNITED STATES PATENTS

2,945,762 7/1960 Carroll et al. .... 96/104  
3,416,927 12/1968 Kalenda .... 96/104

Primary Examiner—J. Travis Brown

Attorney—Sughrue, Rothwell, Mion, Zinn & Macpeak

ABSTRACT: A photographic silver halide emulsion containing at least one sensitizing dye represented by the general formula I



wherein  $\text{Z}_1$  represents a nonmetallic atomic group forming a 4-quinoline nucleus,  $\text{Z}_2$  represents a nonmetallic atomic group necessary to complete a member selected from the group consisting of a 5-membered heterocyclic ring and a 6-membered heterocyclic ring,  $\text{R}_1$  and  $\text{R}_2$  each represents a member selected from the group consisting of a nonsubstituted alkyl group and a substituted alkyl group,  $\text{R}_3$  represents a member selected from the group consisting of a hydrogen atom and an alkylene group condensed with  $\text{R}_2$ ,  $\text{X}$  represents an acid anionic group, and  $p$  and  $m$  each represents 1 or 2, said  $\text{X}$  forming an intramolecular salt when  $p$  is 1, and at least one compound represented by the general



wherein  $\text{D}$  represents a divalent aromatic residual group,  $\text{R}_4$  and  $\text{R}_6$  each represents a member selected from the group consisting of a hydrogen atom, a hydroxyl group, a halogen atom, an alkoxy group, an aryloxy group, and arylthio group,  $\text{R}_5$  represents a member selected from the group consisting of an aryloxy group and an arylthio group, and  $\text{W}$  represents a member selected from the group consisting of  $\text{CH}$  and  $\text{N}$ .

## PHOTOGRAPHIC SILVER HALIDE EMULSION

## BACKGROUND OF THE INVENTION

## 1. Field of the Invention

The present invention relates to a spectral sensitized photographic silver halide emulsion and in particular to a photographic silver halide emulsion in which the formation of photographic fogs caused by the addition of a sensitizing dye is inhibited and the reduction of the color sensitivity during the preservation is prevented.

## 2. Description of the Prior Art

It is well known to spectrally sensitize a photographic silver halide emulsion by incorporating a sensitizing dye in the photographic silver halide emulsion, whereby the range of light-sensitive wavelength is further enlarged to a longer wavelength side. The strength of the spectral sensitization is influenced by the chemical structure of the sensitizing dye to be employed, the properties of the emulsion, such as, the composition of silver halide, the crystal structure of the silver halide, the concentration of silver ion, the pH of the emulsion and the like, as well as the kinds of additives, such as stabilizer, wetting agent, hardening agent and a coupler. Many of the aforesaid additives to be incorporated in a photographic silver halide emulsion together with a sensitizing dye act to weaken the spectral sensitization of the sensitizing dye.

Moreover, although by the addition of a sensitizing dye to a silver halide emulsion, the silver halide emulsion is spectrally sensitized, it usually has a bad influence on the photographic properties of the photographic silver halide emulsion. In particular, the formation of fog caused by the addition of a sensitizing dye (hereinafter, such a fog is called "dye fog") and the instability of the dye sensitivity greatly hinders the preparation of a photographic light-sensitive element having high strength spectral sensitivity, reduced fog and good preservability. When a sensitizing dye is used together with a conventionally employed antifoggant or a stabilizer for improving these drawbacks, the spectral sensitivity is remarkably reduced in some cases. Further, the spectral sensitivity is degraded extremely in other cases when the material is stored. Thus, for obtaining effective results, the aforesaid additives must be selected strictly in accordance with the sensitizing dye to be employed.

An object of the present invention is to provide a photographic silver halide emulsion sensitized by a spectral sensitizing method, in which the formation of dye fogs is inhibited and the degradation of spectral sensitivity with the lapse of time is reduced without lowering the spectral sensitivity.

Another object of the present invention is to provide an excellent red-sensitive silver halide emulsion for color photographic light sensitive materials.

## SUMMARY OF THE INVENTION

According to the present invention, there is provided a photographic silver halide emulsion containing a sensitizing dye represented by the general formula



wherein  $Z_1$  represents a nonmetallic atomic group necessary to complete a 4-quinoline nucleus,  $Z_2$  represents a nonmetallic atomic group necessary to complete a 5-membered or 6-membered heterocyclic ring,  $R_1$  and  $R_2$  each represent an unsubstituted or substituted alkyl group,  $R_3$  represents a hydrogen atom or an alkylene group condensed with said group  $R_2$ ,  $X$  represents an acid anion, and  $p$  and  $m$  each represent 1 or 2, said  $X$  forming an intramolecular salt when  $p$  is 1, and a compound represented by the general formula (II):



wherein D represents a divalent aromatic residual group,  $R_4$  and  $R_6$  each represent a hydrogen atom, a hydroxyl group, a halogen atom, an alkoxyl group, an aryloxyl group, or an arylthio group,  $R_5$  and  $R_7$  each represent an aryloxyl group or an arylthio group, and W represents CH or N.

In General formula I, the 4-quinoline nucleus shown by  $Z_1$  may have a substituent such as a halogen atom, an alkyl group, or an alkoxy group. The examples of the heterocyclic rings to be completed by the nonmetallic atomic group represented by  $Z_2$  are a 4-quinoline nucleus, a 2-quinoline nucleus, a naphthothiazole nucleus, an oxazole nucleus, and a benzimidazole nucleus. Also,  $R_1$  or  $R_2$  may be a lower alkyl group such as a methyl group, an ethyl group or a propyl group or a substituted group thereof such as a  $\beta$ -hydroxyethyl group,  $\beta$ -acetoxyethyl group, or ethylsulfate group; a carboxyalkyl group or a derivative thereof such as a carboxymethyl group or a 2-(2-carboxy-ethoxy) ethyl group; a sulfoalkyl group or a derivative thereof such as a  $\beta$ -sulfoethyl group, a  $\beta$ -sulfopropyl group, or a 3-methoxy-2-(3-sulfopropoxy) propyl group. The main feature of the sensitizing dye having the chemical structure shown by general formula I is that it contains at least one quinoline heterocyclic nucleus.

In general formula II, the examples of the divalent aromatic residual group represented by D are a biphenylene group, a naphthalene group, a stilbene group and a bibenzyl group.

The main feature of the compound represented by general formula II is that each of the pyrimidinylamino nuclei or triazinylamino nuclei bonded by the divalent aromatic residual group has at least one arylthio group or aryl oxy group.

The sensitizing dye represented by general formula I (hereinafter the sensitizing dye is called Sensitizing Dye I) can spectrally sensitize a photographic silver halide emulsion in a wavelength region of from a green region to a red region by 35 properly selecting the heterocyclic nucleus shown by



40 However, there is a fault that in the case of incorporating in a silver halide emulsion the sensitizing dye alone, dye fogs tend to be formed and also the color sensitivity by the sensitizing dye is lowered in course of time.

45 The compound shown by general formula II (hereinafter it  
is called compound II) does not substantially have spectral ab-  
sorption at visible ranges but has a strong absorption at a near  
ultraviolet region. When sensitizing dye I is incorporated in a  
silver halide emulsion together with compound II for sensitiz-  
ing the silver halide emulsion, the formation of dye fogs can be  
50 effectively inhibited and markedly prevented without substan-  
tially reducing the spectral sensitivity. Compound II of this in-  
vention provides the aforesaid merits or effects selectively to  
only the carbocyanine sensitizing dye represented by general  
55 formula I, that is, a sensitizing dye showing a M-band type  
spectral sensitization among various carbocyanine dyes and  
when compound II is incorporated in a photographic silver ha-  
lide emulsion together with other carbocyanine dyes showing  
a J-band type or H-band type spectral sensitization, the spec-  
60 tral sensitivity is markedly reduced on the contrary.

Moreover, among the compounds II used in this invention, the one of which the pyrimidinylamino nuclei each having at least one aryl oxy group or arylthio group has such merits when used together with sensitizing dye I in a photographic silver halide emulsion for color photographic light-sensitive materials that the contamination by color development is prevented, the formation of stains by the sensitizing dye is reduced and the reduction of spectral sensitization by the presence of a coupler is prevented besides the aforesaid spectral sensitivity, and the prevention of the reduction in color sensitivity in course of time.

75 The practical examples of the sensitizing dyes represented by general formula I are shown below although the sensitizing dye is not limited to them only:



Also, the typical examples of the compound represented by General formula II are as follows:



Among the compounds represented by General formula II, the compound in which Z is -N-, that is, the compound having a S-triazine nucleus may be prepared by a well-known method. The compound in which Z is -CH-, that is, having a pyrimidine nucleus may be prepared as follows:

#### PREPARATION I

Mixed with 100 ml. of water and 100 ml. of acetone were 12.4 g. of sodium 4,4'-diaminostilbene-2,2''-disulfonate and 11.0 g. of 2,4,6-trichloropyrimidine and the mixture was stirred at 55°-65°C.

70 The reaction system was maintained to a neutral or weak acid state by neutralizing, with the addition of a 10 percent sodium carbonate solution, hydrochloric acid formed during the reaction. After the reaction was finished, the reaction product mixture was ice-cooled to precipitate a crystal, which 75 was recovered by filtering to provide the compound shown by the following formula IIg.

(IIg)



## PREPARATION 2

## Preparation of Compound IIb

In 70 ml. of dimethylformamide were heated under refluxing for about 2.5 hours 14.1 g. of Compound IIg prepared above, 13.3 g. sodium- $\beta$ -naphtholate, and 1.0 g. of 1,4-diaz-2,2,2-bicyclooctane.

After allowing to cool, the precipitates formed were removed by filtering and the filtrate was subjected to distillation under reduced pressure to remove dimethylformamide. The residue was dissolved in methanol and mixed with about 5 ml. of concentrated hydrochloric acid to deposit a crystal of the objective compound, which was collected by filtering, washed with a small amount of acetone and water, and then dried.

## PREPARATION 3

## Preparation of Compound IIf

In a mixed solvent of 70 ml. of water and 20 ml. of dioxane were heated under refluxing 14.1 g. of compound IIg, 1.0 g. of sodium hydroxide and 4.4 g. of thiophenol. After the reaction was finished, about 5 ml. of concentrated hydrochloric acid was added to the reaction mixture to precipitate the product, which was collected by filtering, washed with water and methanol, and dried.

Sensitizing dye I or compound II in this invention may be incorporated in a silver halide emulsion as an aqueous solution thereof or a solution thereof in a water-soluble solvent such as methanol, ethanol, alkaline methanol, and the like separately, or as a mixture thereof. The amounts thereof and the ratio thereof are suitably selected in accordance with the kinds of each compound, the emulsion to be employed and additives.

A suitable concentration of sensitizing dye I, however, is 0.002-0.2 g. per 1 g. molecule of the silver halide in a silver halide emulsion and a suitable concentration of compound II is 0.01-10 g. per 1 g. molecule of the silver halide in a silver halide emulsion, and a preferable concentration ratio of Sensitizing dye I to compound II is from 1:2 to 1:200.

As the silver halide emulsion used in this invention, there may be used a silver iodo-bromide emulsion, a silver bromide emulsion, a silver chlorobromide emulsion, or a silver chloride emulsion.

The photographic silver halide emulsion may be prepared by a conventional manner and may be applied to a suitable support such as a cellulose derivative film or a baryta coated paper.

Now the invention will further be described by referring to the following practical examples.

## EXAMPLE 1

A definite amount of a  $4 \times 10^{-3}$  mol methanol solution of Sensitizing dye I in this invention was added to 100 g. (AgX:  $33 \times 10^{-3}$  mol) of silver chloro-bromide emulsion prepared by a conventional method and a definite amount of a 0.1 percent methanol solution of compound II was immediately added to the resulting emulsion. The mixture was stirred for 1 hour at 40° C. and applied to a support in a thickness of 7 ml. per cabinet size followed by drying.

The light sensitive element thus prepared was exposed by using an optical wedge through a blue filter transmitting only light having shorter wavelengths than 500 m.  $\mu$  and a yellow filter transmitting only light having longer wavelengths than 500 m.  $\mu$  and then developed for 10 minutes at 20° C. in a

5 developer having the composition shown below, followed by fixing.

|    |                                   |         |
|----|-----------------------------------|---------|
| 5  | Metol                             | 0.3 g.  |
|    | Potassium Pyrosulfite             | 1.4 g.  |
|    | Sodium Sulfite (anhydrous)        | 38 g.   |
|    | Hydroquinone                      | 6 g.    |
|    | Sodium Carbonate<br>(Monohydrate) | 22.5 g. |
| 10 | Potassium Bromide                 | 0.9 g.  |
|    | Citric Acid                       | 0.7 g.  |
|    | Water To Make                     | 100 ml. |

For the thus developed light sensitive element, the density, the blue sensitivity ( $S_B$ ) using a blue filter, and the spectral sensitivity ( $S_{SPC}$ ) using a yellow filter were measured, the results of which are shown in table 1.

| Experiment Number | Sensitizing dye | Amt. (ml.) | Compound II | Filter relative sensitivity |       |           |
|-------------------|-----------------|------------|-------------|-----------------------------|-------|-----------|
|                   |                 |            |             | Amt. (ml.)                  | $S_B$ | $S_{SPC}$ |

TABLE 1

| Experiment Number | Sensitizing dye | Amt. (ml.) | Compound II | Filter relative sensitivity |       |           |
|-------------------|-----------------|------------|-------------|-----------------------------|-------|-----------|
|                   |                 |            |             | Amt. (ml.)                  | $S_B$ | $S_{SPC}$ |
| 20                | .....           | .....      | .....       | 0.0                         | 100   | 0         |
| 30                | 1A              | 1.0        | IIa         | .....                       | 100   | 100       |
|                   |                 | 2.0        |             | .....                       | 100   | 141       |
|                   |                 | 4.0        |             | .....                       | 71    | 141       |
|                   |                 | 2.0        |             | 4                           | 117   | 200       |
| 35                | 2               | 2.0        | IIB         | 8                           | 110   | 200       |
|                   |                 | 2.0        |             | 4                           | 117   | 200       |
|                   |                 | 2.0        |             | 8                           | 117   | 200       |
| 40                | 1B              | 1.0        | III         | .....                       | 90    | 300       |
|                   |                 | 2.0        |             | .....                       | 85    | 340       |
|                   |                 | 1.0        |             | 4                           | 100   | 345       |
|                   |                 | 1.0        |             | 8                           | 115   | 350       |
| 45                | 4               | 1.0        | IIc         | .....                       | 95    | 170       |
|                   |                 | 2.0        |             | .....                       | 71    | 200       |
|                   |                 | 2.0        |             | 4                           | 117   | 282       |
|                   |                 | 2.0        |             | 8                           | 125   | 316       |
| 50                | 5               | 1.0        | IId         | .....                       | 110   | 214       |
|                   |                 | 2.0        |             | .....                       | 117   | 225       |
|                   |                 | 2.0        |             | 4                           | 125   | 320       |
|                   |                 | 2.0        |             | 8                           | 125   | 320       |
| 55                | 6               | 1.0        | IIe         | .....                       | 100   | 170       |
|                   |                 | 2.0        |             | .....                       | 100   | 170       |
|                   |                 | 4.0        |             | .....                       | 70    | 200       |
|                   |                 | 2.0        |             | 4                           | 100   | 220       |
| 60                | 7               | 2.0        | IIe         | 8                           | 100   | 235       |
|                   |                 | 2.0        |             | 4                           | 110   | 340       |
|                   |                 | 2.0        |             | 8                           | 110   | 340       |
|                   |                 | 2.0        |             | 8                           | 117   | 400       |
| 70                | 8               | 2.0        | IIIf        | 4                           | 110   | 282       |
|                   |                 | 2.0        |             | 8                           | 117   | 400       |

From the above results, it will be understood that by incorporating in a photographic light sensitive emulsion Sensitizing dye I and compound II simultaneously, the color sensitivity of the emulsion is increased and the formation of fogs is inhibited.

## EXAMPLE 2

A definite amount of a  $4 \times 10^{-3}$  mol methanol solution of Sensitizing dye I and a definite amount of a 0.1 percent methanol solution of compound II were added to 100 g. (AgX:  $30 \times 10^{-3}$  mol) of a silver bromide emulsion prepared by a conventional method. The resulting emulsion was stirred for 30 minutes at 40° C., mixed with a hardening agent and a wetting agent, and applied to a film base followed by drying.

The light sensitive film was stored at a temperature of 24°-30 C. and a relative humidity of 65-70 percent and the spectral sensitivity ( $S_{SPC}$ ) using a yellow filter was measured as in example 1, the results of which are shown in table 2.

TABLE 2

| Experiment No. | Sensitizing dye | Amt. (ml.) | Compound II | Amt. (ml.) | Filter relative sensitivity, Sspc |               |               |
|----------------|-----------------|------------|-------------|------------|-----------------------------------|---------------|---------------|
|                |                 |            |             |            | Directly after coating            | After 1 month | After 4 month |
| 9----- IA      |                 | 2.0        |             | 0          | 100                               | 65            | 50            |
|                |                 | 2.0        | IIa         | 4          | 200                               | 150           | 135           |
|                |                 | 2.0        |             | 8          | 200                               | 185           | 173           |
| 10----- IC     |                 | 2.0        |             | 0          | 100                               | 85            | 75            |
|                |                 | 2.0        | IIb         | 4          | 141                               | 138           | 100           |
|                |                 | 2.0        |             | 8          | 200                               | 198           | 188           |
| 11----- IE     |                 | 2.0        |             | 0          | 100                               | 73            | 60            |
|                |                 | 2.0        | IIc         | 4          | 200                               | 160           | 130           |
|                |                 | 2.0        |             | 8          | 200                               | 167           | 151           |
| 12----- ID     |                 | 2.0        |             | 0          | 100                               | 83            | 80            |
|                |                 | 2.0        | IId         | 4          | 141                               | 110           | 110           |
|                |                 | 2.0        |             | 8          | 141                               | 138           | 128           |

We claim:

wherein A photographic silver halide emulsion containing at least one sensitizing dye represented by the following general formula: 20



wherein  $Z_1$  represents a nonmetallic atomic group forming a nucleus of the 4-quinoline series,  $Z_2$  represents a nonmetallic atomic group necessary to complete a member selected from the group consisting of a 4-quinoline nucleus, a 2-quinoline nucleus, a naphthothiazole nucleus, an oxazole nucleus, and a benzimidazole nucleus,  $R_1$  and  $R_2$  each represents a member selected from the group consisting of an alkyl group, a hydroxyl group, an acetoxyalkyl group, an alkylsulfate group, a carboxyalkyl group, a carboalkoxyalkyl group, a sulfoalkyl group, an alkoxy sulfoalkoxyalkyl group,  $R_3$  represents a member selected from the group consisting of a hydrogen atom and an alkylene group having 2-5 carbon atoms capable of condensing with  $R_2$ ,  $X$  represents an acid anionic group, and  $P$  and  $m$  each represents 1 or 2, said  $X$  forming an in-40  
tramolecular salt when  $P$  is 1, and at least one compound represented by the following general formula:



wherein D represents a divalent aromatic residual group selected from the group consisting of a biphenylene group 50



a phenylene group



a naphthylene group ( $-\text{C}_{10}\text{H}_7-$ ), a stilbene group



and a bibenzyl group



$R_4$  and  $R_6$  each represents a member selected from the group consisting of a hydrogen atom, a hydroxyl group, a halogen atom, an alkoxy group, an aryloxy group and arylthio group. 75

$R_5$  and  $R_7$  each represents a member selected from the group consisting of an aryloxyl group and an arylthio group, and  $W$  represents a member selected from the group consisting of  $CH$  and  $N$ .

5 2. The photographic silver halide emulsion as claimed in  
claim 1 wherein said sensitizing dye is a compound selected  
from the group consisting of:



and



60 3. The photographic silver halide emulsion as claimed in claim 1 wherein said compound represented by general formula II is selected from the group consisting of:





4. The emulsion of claim 1 wherein said D is substituted with an  $-SO_3M$  group, where M is selected from the group consisting of a hydrogen atom and a metal which forms a water-soluble salt.

5. The emulsion of claim 1 wherein said silver halide is selected from the group consisting of silver iodobromide, 40 silver bromide, silver chlorobromide and silver chloride.

6. The photographic silver halide emulsion as claimed in claim 1, wherein the concentration of said sensitizing dye is 0.002-0.2 g. per gram molecule of the silver halide.

45 7. The photographic silver halide emulsion as claimed in claim 1, wherein the concentration of said compound represented by the general formula II is 0.02-10 g. per gram molecule of the silver halide.

8. The photographic silver halide emulsion as claimed in claim 1, wherein the concentration ratio of said sensitizing dye of formula I to said compound represented by the general formula II is from 1:2 to 1:200.

.55

60

65

70

75